

July 3, 1962

G. R. HEMMETER

3,042,556

PROCESS FOR TREATING STEEL

Filed Feb. 2, 1960

5 Sheets-Sheet 1

FIG. 1.

2.85% SILICON STEEL STRIP  
ANNEALED AT TEMPERATURE OF 1650° FARENHEIT



Inventor:  
George R. Hemmeter,

by Henry J. Marcinko  
Attorney.

July 3, 1962

G. R. HEMMETER

3,042,556

PROCESS FOR TREATING STEEL

Filed Feb. 2, 1960

5 Sheets-Sheet 2

Fig. 2.  
2.85% SILICON STEEL STRIP MAGNETICALLY  
ANNEALED AT TEMPERATURE OF 1750° FAHRENHEIT



Inventor:  
George R. Hemmeter;

by Harry J. Mannion  
Attorney.

July 3, 1962

G. R. HEMMETER

3,042,556

PROCESS FOR TREATING STEEL

Filed Feb. 2, 1960

5 Sheets-Sheet 3

FIG. 3.

2.85% SILICON STEEL STRIP - CORE LOSSES  
MEASURED AT A FLUX DENSITY OF 15 KILOGAUSS

% ELONGATION

CORE LOSS (WATTS PER POUND)



% ELONGATION

CORE LOSS (WATTS PER POUND)

INVENTOR:  
George R. Hemmeter,

by Mary J. Marinick  
Attorney.



1900

1800

1700

1600

1500

1400

July 3, 1962

G. R. HEMMETER  
PROCESS FOR TREATING STEEL

3,042,556

Filed Feb. 2, 1960

5 Sheets-Sheet 4

FIG. 4.



Inventor:  
George R. Hemmeter,

by Harry J. Marinich  
Attorney.

July 3, 1962

G. R. HEMMETER

3,042,556

PROCESS FOR TREATING STEEL

Filed Feb. 2, 1960

5 Sheets-Sheet 5



Inventor:  
George R. Hemmeter

by Henry J. Marinino  
Attorney.

## 1

3,042,556

## PROCESS FOR TREATING STEEL

George R. Hemmeter, Fort Wayne, Ind., assignor to General Electric Company, a corporation of New York  
Filed Feb. 2, 1960, Ser. No. 6,190  
4 Claims. (Cl. 148—111)

This invention relates to a process for treating electrical steel, and in particular, to a process which is adaptable for a production line type of operation for manufacturing laminations and core components for dynamoelectric machines from a critically strained silicon steel strip. This application is a continuation-in-part of my application Serial Number 667,947, filed June 25, 1957, now abandoned.

Conventional methods of producing laminations and core components have not been satisfactory from an economic standpoint to adapt to a production line operation. A principal drawback has been the comparatively long periods of time required to accomplish magnetic annealing of the fabricated parts. Heretofore, it has been the practice in industry to carry out the magnetic anneal of critically strained silicon steel strips in roller hearth furnaces requiring a semibatch type of operation. There is therefore a need in industry for a magnetic annealing treatment with a time rate of relatively short duration that will bring about the requisite change in grain structure necessary for improving the magnetic quality and thereby make it practicable to produce laminations and core components on a continuous production line basis.

A typical critically strained silicon steel strip that can be employed in the practice of the invention is described in the McKnight Patent 2,738,295, granted on March 13, 1956. The improved magnetic characteristics of such critically strained silicon steels when subjected to a magnetic anneal are well known.

A principal purpose of the magnetic annealing treatment is to obtain a grain orientation and size which will improve the magnetic quality of the steel and the improved magnetic properties are not obtained in this steel until the completely new grain structure is formed. It will be appreciated that an annealing treatment for magnetic properties differs from the conventional annealing methods employed to improve mechanical properties of a steel, such as its ductility, since the improvement in the mechanical properties may not necessarily bring about the desired improvement in the magnetic quality of the steel. In the past, to produce the grain structure requisite for minimum core losses, the annealing time was generally on the order of an hour or more at temperature, and for this reason the magnetic annealing treatment was carried out in large furnaces in a semi-batch type of operation. It is therefore desirable that the magnetic annealing be accomplished in relatively shorter periods of time so that a heating means readily adaptable to a production line operation, such as induction heating, may be effectively employed. Thus, by making it possible to utilize induction heating techniques and the like the advantages of lower capital investment, reduced floor space, lower maintenance costs, decreased amounts of handling and lower production costs can be realized.

In the application of magnetic steels, it is also necessary that consideration be given to the mechanical properties of the steel during its processing. Generally, the surface of the laminations fabricated from an electrical steel strip should be relatively smooth in order that a high space factor may be obtained when the laminations are stacked. In a critically strained electrical steel strip, because of the deformation present in the strip, it is desirable that any residual stresses which might have an

## 2

adverse effect upon magnetic or mechanical properties or result in a distortion of the strip be eliminated.

A general object of the present invention is to provide an improved method for magnetically annealing critically strained silicon steel strip.

It is another object of the invention to provide an improved method of magnetic annealing that is readily adaptable to a production line manufacturing operation.

A further object of the invention is to provide an improved process of treating an electrical steel strip in which the magnetic annealing of the steel strip can be accomplished in relatively short periods of time to produce a steel strip of improved magnetic quality.

In accordance with the invention, a process of treating a silicon steel strip is provided wherein it is conditioned so that a minimum core loss can be achieved by an annealing treatment which requires a total isothermal heating time ranging from 15 seconds to 15 minutes. A silicon steel strip of a thickness ranging from .05 to .125 inch is cold rolled to an intermediate thickness which requires a predetermined elongation from 2 percent to 12 percent elongation to bring the thickness down to desired final gauge.

After this cold reduction, the steel strip is subjected to a normalizing treatment and cooled. After this step, the critically strained strip may be fabricated into the desired shape for the particular electrical application in which it is intended. The parts are then magnetically annealed at the minimum time ranging between 15 seconds and 15 minutes at a preselected isothermal annealing temperature between 1650 degrees and 2100 degrees Fahrenheit that will result in a 100 percent grain response or minimum core loss.

Unexpectedly, it was found that for a fixed magnetic annealing time the lowest temperature within the foregoing temperature range that produces a 100 percent grain response also produces the largest grain structure and the lowest core loss obtainable at the fixed annealing time. Contrary to what might be expected, to carry out the magnetic annealing treatment at a higher temperature for the aforementioned fixed annealing time produced a grain structure that provided an increased core loss. Thus, for a fixed predetermined annealing time a minimum core loss is obtained at approximately the same time that the 100 percent grain response is achieved at the lowest isothermal annealing temperature required for the predetermined annealing time.

As the term is used herein, 100 percent grain response means that the microstructure of the material does not contain a matrix of fine grained material, but one in which the fine grains have been consumed by the larger growing grains as evidenced by an examination of representative photomicrographs of the material.

Further objects and advantages of this invention will become apparent and the invention will be better understood by reference to the following description and the accompanying drawings in which:

FIG. 1 shows comparative curves illustrating the variation in core loss with flux density for a 2.85 percent silicon steel strip with a 4 percent elongation and for the same steel with a 10 percent elongation, both annealed at a temperature of 1650 degrees Fahrenheit at fixed annealing times of  $\frac{1}{2}$ , 1,  $2\frac{1}{2}$  and 5 minutes;

FIG. 2 shows comparative curves illustrating the variation in core loss with changes in flux density for a 2.85 percent silicon steel strip with a 4 percent elongation and for the same steel with a 10 percent elongation, both annealed at a temperature of 1750 degrees Fahrenheit at fixed annealing times of  $\frac{1}{2}$ , 1,  $2\frac{1}{2}$  and 5 minutes;

FIG. 3 shows comparative curves illustrating the core loss versus temperature for a 2.85 percent silicon steel

strip with a 4 percent elongation and for the same steel with a 10 percent elongation for fixed annealing times of  $\frac{1}{2}$ , 1,  $2\frac{1}{2}$  and 5 minutes;

FIG. 4 shows the curves illustrating reduction of core loss plotted against temperature for a 3.06 percent silicon steel strip with a 4 percent elongation for fixed annealing times of  $\frac{1}{2}$ , 1,  $2\frac{1}{2}$ , 5 and 10 minutes;

FIG. 5 is a graph setting forth the percent grain response of a 1.5 percent silicon steel strip with a 4 percent elongation at different temperatures for fixed time intervals of 15 seconds, 30 seconds, 1 minute, 5 minutes and 15 minutes; and

FIG. 6 is a graph setting forth the average grain size plotted against time and temperature for an annealed 1.5 percent silicon steel strip with a 4 percent elongation.

The silicon strip steel used in the practice of the invention is made from ingots melted in an open hearth or electric furnace and preferably has a silicon content between 0.25 and 3.5 percent by weight and a manganese content between .20 and .40 percent by weight. Aluminum may be present in an amount between .02 and .60 percent by weight. It is preferable that the phosphorus and carbon content be kept down below .05 percent. A maximum of .03 percent of sulphur may be present in the composition.

An ingot having the desired composition is heated in a soaking pit in the mill and hot rolled into slabs of the width of the finished coil and of a thickness between 0.05 and .125 inch, depending upon the final gauge to which the steel strip will ultimately be rolled. After the hot roll, it is passed through a pickling bath to remove any scale produced by the hot rolling operation. The steel strip is then given a cold reduction to reduce the strip to an intermediate thickness which will require a predetermined elongation ranging from 2 to 12 percent to bring the strip down to its final desired gauge. The first mill pass or first cold reduction of the silicon steel strip is of significance in the practice of the present invention since it affects the second cold reduction step with which this invention is more particularly concerned and which, as hereinafter will be more fully described, is a factor that affects the rate of the annealing treatment.

After completion of the first mill pass or cold reduction, the steel strip is given a normalizing treatment. The strip is passed through a furnace for a sufficient length of time to achieve a recrystallization. The normalizing temperature, as the term is used herein, is the temperature equal to or above the recrystallization temperature for the particular silicon steel, which is required to achieve recrystallization of the steel but precludes substantial grain growth. The temperature of recrystallization may vary from 1500 to 1850 degrees Fahrenheit depending upon the specific composition of the silicon steel strip. The time required will vary from 2 to 8 minutes depending upon the gauge of the strip and the temperature of the furnace. The purpose of the normalizing treatment is to recrystallize the fragmented grains of the deformed steel and produce a steel having a very fine equiaxed grain structure.

The normalized silicon steel strip is then subjected to a final cold pass or cold reduction to produce the final gauge of the strip. It will be appreciated that the hereinbefore described steps can be readily carried out at the mill in accordance with the specifications of the electrical equipment manufacturer. In this condition, the steel strip is ready for fabrication into laminations and the like.

After fabrication by the manufacturer, the silicon steel strip has been subjected to a severe straining which results from the shearing, punching and stamping operation performed upon the strip. Heretofore, it has not been considered possible to anneal such silicon steel strips in relatively short intervals of time or to obtain the requisite grain structure required in steels of high magnetic quality that would make it possible to carry out the annealing in a production line type of manufacturing operation. In the past, it was considered necessary to heat the fabricated elements for relatively long periods at temperatures above

1400 degrees Fahrenheit to relieve the stresses and achieve the requisite grain structure.

It was found that the steels containing from .25 to 3.5 percent silicon critically strained in the final cold reduction in accordance with the present invention can be annealed in relatively short intervals of time ranging from 15 seconds to 15 minutes. Further, it was found that a silicon steel processed for a 10 percent elongation, as compared with a 4 percent elongation, could be annealed in a shorter period of time or at a reduced annealing temperature. In either case, the time intervals involved are short enough to permit the annealing to be carried out in a continuous production line type of operation. Further, it will be appreciated that additional advantages afforded by a lower temperature of magnetic annealing are that difficulties encountered with adjacent layers of laminations sticking can be minimized and savings in energy requirements due to the lower temperature can be realized.

The curves of FIG. 1 of the drawings illustrate the comparative effect of a 4 percent and a 10 percent elongation on core loss of the silicon steel strip at a temperature of 1650 degrees Fahrenheit. FIG. 2 illustrates the corresponding curves at a temperature of 1750 degrees Fahrenheit. From these curves, it will be seen that the steel strips with the 10 percent elongation produced by the final mill pass are more responsive to annealing than the strips with the 4 percent elongation. For the 2.85 percent silicon steel strips used, it was found that at a temperature between 1600 and 1700 degrees Fahrenheit the response for the steel having the 10 percent elongation was five times as fast as the identical strip with the 4 percent elongation. It will be seen from FIG. 1 that at 1650 degrees Fahrenheit all of the sample strips, which were subjected to a mill pass producing the 10 percent elongation, are completely annealed as evidence by the close grouping of all the curves. However, the curves for the steel strip samples with the 4 percent elongation indicate that only the 5 minute annealing time has produced a desirable grain structure and acceptable magnetic quality. Further, it will be apparent that for annealing times as short as one-half minute, a steel strip with 4 percent elongation requires a temperature of at least 1750 degrees Fahrenheit before a complete grain response can be obtained.

In the curves of FIG. 3, the magnetic annealing response of the 2.85 percent silicon steel strip, as it is affected by temperature, is graphically shown. However, it will be noted that values given are for a single flux density of 15 kilogausses. From these curves, it can be seen that at 1500 degrees Fahrenheit the steel strips with a 10 percent elongation have already begun to be annealed as evidenced by the reduction in core loss for the  $2\frac{1}{2}$  and 5 minute fixed time intervals. However, the silicon steel strips with a 4 percent elongation show no signs of being annealed at 1500 degrees Fahrenheit for any of the fixed time intervals. At the 1800, 1850 and 1900 degrees Fahrenheit temperature levels, there is no substantial change in core loss. Contrary to what might be expected, it will be seen from the curves of FIG. 3 that the minimum core losses occur at a relatively low temperature for each of the illustrated fixed time curves as indicated by temperatures at the minimal points of the curves. This prolonged heating above the temperature which corresponds to the minimum core loss will result in an increased core loss. Thus, for the strip with a 10 percent elongation the minimum core loss occurs at 1600 degrees for a fixed annealing period of  $2\frac{1}{2}$  minutes. If the magnetic anneal is carried out at 1800 degrees Fahrenheit for the  $2\frac{1}{2}$  minutes fixed interval, it will be seen from the curve of FIG. 3 that the core losses are increased. Further, the curves indicate that the minimum core losses obtainable from a 4 percent or 10 percent final mill pass are approximately the same but are achieved under different time and temperature annealing conditions for each of the magnetic materials. The effect of the elongation produced by the final mill pass is to shift the group of curves for a specific

elongation to the left, as viewed in FIG. 3, as the elongation is increased as high as 12 percent.

For the silicon steel strips with 10 percent elongation, an annealing temperature between 1650 and 1850 degrees Fahrenheit will produce satisfactory magnetic properties for the periods of time preselected in accordance with this invention. As previously mentioned, the lower temperature can be utilized to an advantage in production line operation to minimize the tendency of the laminations to stick together during the magnetic annealing treatment and to achieve economies in the amount of energy required to effect the magnetic anneal treatment. If such an advantage is not of a significant factor, by increasing the annealing temperature, the annealing time can be reduced with a resultant increase in productive output.

The silicon steel strips used to obtain the data for the curves of FIGS. 1, 2 and 3 were of the following composition as determined by chemical analysis.

| Constituent: | Percent by weight |
|--------------|-------------------|
| Silicon      | 2.85              |
| Carbon       | .024              |
| Aluminum     | .23               |
| Manganese    | .290              |
| Phosphorus   | .01               |
| Sulphur      | .024              |
| Nickel       | .06               |
| Copper       | .07               |
| Tin          | .01               |

perature at fixed times for a silicon steel having the following analysis.

| Constituent: | Percent by weight |
|--------------|-------------------|
| Silicon      | 3.06              |
| Carbon       | .025              |
| Aluminum     | .26               |
| Manganese    | .33               |
| Phosphorus   | .008              |
| Sulphur      | .025              |
| Nickel       | .13               |
| Copper       | .071              |
| Tin          | .011              |

A steel strip of the foregoing composition was given a final mill pass which produced a 4 percent elongation at a final gauge of .025 inch. In order to obtain the data for the purpose of FIG. 4, rectangular laminations  $1\frac{3}{16}$  inch wide and 4 inches long were cut with the longer dimension in the rolling direction. The strips were properly identified and were subjected to an annealing treatment for fixed times of  $\frac{1}{2}$ ,  $2\frac{1}{2}$ , 5 and 10 minutes at 50 degree temperature intervals of from 1500 degrees to 1900 degrees Fahrenheit. Core loss measurements at a flux density of 10 kilogausses were taken for both annealed and unannealed magnetic samples. The core losses of the unannealed sample laminations are presented in Table I and the core losses of the annealed laminations are presented in Table II.

TABLE I  
Average Core Losses of Single Strips Before Annealing  
(Watts Per Pound) at 10 Kilogausses

| Minutes               | 1,500<br>°F. | 1,550<br>°F. | 1,600<br>°F. | 1,650<br>°F. | 1,700<br>°F. | 1,750<br>°F. | 1,800<br>°F. | 1,850<br>°F. | 1,900<br>°F. |
|-----------------------|--------------|--------------|--------------|--------------|--------------|--------------|--------------|--------------|--------------|
| 10.....               | 2.617        | 2.633        | 2.583        | 2.637        | 2.617        | 2.620        | .....        | .....        | .....        |
| 5.....                | 2.677        | 2.630        | 2.653        | 2.633        | 2.610        | 2.647        | .....        | .....        | .....        |
| 2 $\frac{1}{2}$ ..... | 2.640        | 2.613        | 2.680        | 2.657        | 2.657        | 2.660        | 2.647        | .....        | .....        |
| 1.....                | 2.637        | 2.637        | 2.657        | 2.657        | 2.657        | 2.667        | 2.643        | 2.643        | 2.643        |
| $\frac{1}{2}$ .....   | .....        | .....        | 2.607        | 2.657        | 2.643        | 2.667        | 2.643        | 2.643        | 2.643        |

TABLE II  
Average Core Losses of Single Strips After Annealing  
(Watts Per Pound) at 10 Kilogausses

| Minutes               | 1,500<br>°F. | 1,550<br>°F. | 1,600<br>°F. | 1,650<br>°F. | 1,700<br>°F. | 1,750<br>°F. | 1,800<br>°F. | 1,850<br>°F. | 1,900<br>°F. |
|-----------------------|--------------|--------------|--------------|--------------|--------------|--------------|--------------|--------------|--------------|
| 10.....               | 1.647        | 1.20         | .837         | .937         | .900         | .....        | .....        | .....        | .....        |
| 5.....                | 1.517        | 1.16         | .00          | .92          | .92          | .....        | .....        | .....        | .....        |
| 2 $\frac{1}{2}$ ..... | 1.553        | 1.287        | .85          | .927         | .92          | .....        | .....        | .....        | .....        |
| 1.....                | 1.603        | 1.29         | .903         | .913         | .923         | .....        | .....        | .....        | .....        |
| $\frac{1}{2}$ .....   | .....        | 1.627        | 1.607        | 1.157        | .927         | .....        | .....        | .....        | .....        |

A steel strip of the foregoing composition was given a final mill pass that produced a 4 percent elongation and another steel strip of the same composition was given a mill pass that produced a 10 percent elongation. The final thickness of the steel strip having the 4 percent elongation was 24.8 mils and the final thickness of the material having the 10 percent elongation was 23.6 mils. The two steel strips were cut into rectangular laminations 4 inches long and  $1\frac{3}{16}$  inch wide with the rolling direction parallel to the 4 inch dimension. The fixed annealing times, used at each 50 degree temperature interval between 1500 degrees Fahrenheit to 1900 degrees Fahrenheit, were  $\frac{1}{2}$ , 1,  $2\frac{1}{2}$  and 5 minutes. Three laminations were annealed at each combination of time and temperature and the laminations with the 4 percent and the 10 percent elongations were given identical annealing treatments.

As a further illustration of the improvement obtained by practicing the process of this invention, the curves of FIG. 4 show a plot of reduction of core loss versus tem-

60 Referring to FIG. 4, it will be noted that the reduction of core loss of the sample laminations annealed in accordance with the present invention reach a peak or minimum core loss and then decrease. From these curves, it can be readily seen that sample laminations which were annealed at lower temperatures require longer times to reach their minimum core loss level, while those annealed at higher temperatures require shorter annealing times to reach approximately the same level. According to the 65 present invention, the preferred times and temperatures for annealing the 3.06 percent silicon steel strip used in this exemplification of the invention are as follows.

| Temperature by<br>70 degrees Fahrenheit: | Time required<br>(minutes) |
|------------------------------------------|----------------------------|
| 1850                                     | $\frac{1}{2}$              |
| 1750                                     | 1                          |
| 1700                                     | $2\frac{1}{2}$             |
| 1650                                     | 5                          |
| 1600                                     | 5                          |

It is to be understood that the times presented are for a silicon steel strip subject to a final mill pass that produced a 4 percent elongation. However, further reductions in time can be obtained by a final mill pass that will produce a strip having an elongation at final gauge greater than 4 percent. It will be appreciated that the annealing times given in FIG. 4 are minimum times at an isothermal annealing temperature. Depending on the thickness of the strip and method of heating, sufficient time must be allowed for the entire mass to come up to temperature before the specified times apply.

In carrying out the foregoing investigations of the effect of the various factors on the annealing time, it was found that for a fixed annealing time the lowest temperature which produced a 100 percent grain response also produced the largest grains and the lowest core loss obtainable for such an annealing time. Annealing at a higher temperature than required for a given annealing time also produced a 100 percent response but the grains became smaller and the core loss increased. In other words, I have found that minimum core loss is achieved at approximately the same time that a 100 percent grain response is initially obtained.

In the curves of FIG. 5 the relationship between percent grain response and temperature at fixed annealing times is graphically shown for a 1.5 percent silicon steel. In the curve of FIG. 6 the diameter of the average grain size in millimeters is plotted against annealing temperature. The 1.5 percent silicon steel strip used to obtain the data for the curves in FIGS. 5 and 6 was given a final mill pass to produce approximately a 4 percent elongation and was cut in rectangular laminations  $1\frac{1}{2}$  inches long and  $1\frac{3}{16}$  inches wide. The final gauge of the strip was .025 inch. The sample laminations were heated at temperatures of 1600, 1700, 1750, 1800, 1850 and 1900 degrees Fahrenheit for a time interval at each temperature of 15 seconds, 30 seconds, 1 minute, 5 minutes, 15 minutes, 30 minutes and 60 minutes. After each treatment, the sample laminations were air cooled to room temperature, washed clean with water and macroetched in a 30 percent nitric acid solution. The percent area covered by large grains was ascertained by visual inspection and the average grain size of the grains was measured across their average diameter.

From the curves of FIG. 5 it will be seen that a 100 percent grain response or minimum core loss can be obtained by magnetically annealing the 1.5 percent silicon steel strip having a 4 percent elongation at the following times of temperatures.

| Temperature by degrees Fahrenheit: | Time required |
|------------------------------------|---------------|
| 2000                               | seconds 15    |
| 1900                               | do 30         |
| 1850                               | minutes 1     |
| 1800                               | do 5          |

It will be appreciated that the short magnetic annealing times required in accordance with the present invention make it possible for the fabricated electric parts to be heated by high frequency induction methods in a production line type of operation and is the preferred method of heating. If flame heating is to be used or if it is to be carried out by passing the material through a conventional furnace, it is necessary to maintain a small number of layers as the parts formed of the strip are continuously fed to the heating means. The parts should not be very far removed from an outer surface of the layers so that the heat can effectively penetrate all the parts. High frequency induction heating is preferred since such heating results in the generation of heat from within the part and thereby quickly brings the material up to the required temperature.

Referring now to FIG. 6, it will be seen that as the temperature increases and the time required for a 100 percent grain response decreases, the grain size will also

decrease. The decrease in grain size from the 15 minute time interval to the 15 second time interval is relatively small for the 1.5 percent silicon steel. It was found for this steel that a temperature of 1850 degrees Fahrenheit and a magnetic annealing time of 1 minute produced uniformly improved magnetic properties since the time interval could be accurately controlled.

The exact mechanism of the magnetic annealing treatment of the present invention is not clearly understood but is based on strain induced grain boundary migration. The outstanding factor of the mechanism is that abnormal grain size is obtained in comparatively short periods of time. It is clear that conventional steels would require extremely long periods of time and temperature to produce the magnetic properties achieved by the anneal of this invention. It is believed that the final grain size is dependent to a large extent upon the number of active growth sites which are nucleated. The annealing treatment, all other factors being equal, does not depend upon additional grain growth following complete grain response as in the case of normal recrystallization. The extremely fast rate of abnormal grain growth can be attributed to the fact that the growing grains, prior to the 100 percent grain response are consuming a relatively fine grained high energy matrix. Such a mechanism differs from the grain growth that takes place in a completely recrystallized structure in which a substantially lesser driving force is available for the reaction because of the greater uniformity of the grain size and greater equality of the energy levels.

While this invention has been explained by describing several exemplifications thereof, it will be apparent that improvements and modifications may be made without departing from the spirit and scope of the invention as defined in the appended claims.

What I claim as new and desire to secure by Letters Patent of the United States is:

1. A process of treating silicon strip steel having a silicon content between 0.25 percent and 3.5 percent and hot rolled to a thickness between .05 and .125 inch, said process comprising the steps of: cold rolling said strip to an intermediate thickness which when reduced to final gauge will produce a predetermined elongation between 2 and 12 percent in the strip, heating said strip at a normalizing temperature for a period sufficient to effect recrystallization without appreciable grain growth, cold rolling said strip to final gauge, and annealing said strip at a temperature ranging from 1650 to 2100 degrees Fahrenheit for a predetermined period of time ranging from 15 seconds to 15 minutes at a temperature which will produce a minimum core loss for said predetermined period of time and said predetermined elongation, increasing said elongation causing a decrease in the annealing temperature required to produce said minimum core loss.

2. A process of treating a strip steel hot rolled to a thickness ranging from .05 to .125 inch and having a silicon content between 0.25 percent and 3.5 percent, said process comprising: cold rolling said strip to an intermediate thickness requiring a predetermined elongation from 2 to 12 percent to reduce said thickness to final gauge, heating said strip at a normalizing temperature for a sufficient period of time to effect recrystallization without any appreciable grain growth, cooling said strip, cold rolling said strip to final gauge and heating said strip at a temperature ranging from 1650 to 2100 degrees Fahrenheit for a preselected period of time ranging from 15 seconds to 15 minutes at the lowest temperature required to produce a minimum core loss for said preselected period of time and said predetermined elongation, increasing said elongation causing a decrease in the annealing temperature required to produce said minimum core loss.

3. A process of treating a silicon steel strip hot rolled

to a thickness ranging from .05 to .125 inch and having a silicon content between 0.25 percent and 3.5 percent comprising the steps of: cold rolling said strip to an intermediate thickness requiring a predetermined elongation ranging from 2 to 12 percent to reduce said thickness to final gauge, heating said strip at a normalizing temperature for a period long enough to effect recrystallization without any appreciable grain growth, cooling said strip, cold rolling said strip to final gauge, and annealing said strip at a temperature ranging from 1650 to 2100 degrees Fahrenheit for a preselected period of time ranging from 15 seconds to 15 minutes at approximately the lowest temperature required to produce a minimum core loss corresponding to said preselected period of time and said predetermined elongation, increasing said elongation causing a decrease in the annealing temperature required to produce said minimum core loss.

4. A process of treating silicon strip steel hot rolled to a thickness ranging between .05 and .125 inch and having a silicon content from 0.25 to 3.5 percent comprising the steps of: cold rolling said strip to an intermediate thickness requiring approximately 10 percent elongation to reduce said strip to final gauge, heating

said strip at a normalizing temperature for a period sufficient to effect recrystallization without appreciable grain growth and then cooling said strip, cold rolling said strip to final gauge, and annealing said strip for approximately 1 minute at a temperature ranging from 1650 to 1850 degrees Fahrenheit that will produce a minimum core loss corresponding to said elongation and said annealing period, increasing said elongation causing a decrease in the annealing temperature required to produce minimum core loss.

## References Cited in the file of this patent

## UNITED STATES PATENTS

|    |           |                  |               |
|----|-----------|------------------|---------------|
| 15 | 2,287,467 | Carpenter et al. | June 23, 1942 |
|    | 2,378,321 | Pakkala          | June 12, 1945 |
|    | 2,738,295 | McKnight et al.  | Mar. 13, 1956 |
|    | 2,867,558 | May              | Jan. 6, 1959  |

## OTHER REFERENCES

- 20 Engineering Metals and Their Alloys, Samans, The Macmillan Co., N.Y., 1949 (pp. 92-94 relied upon).  
 A Dictionary of Metallurgy, A. D. Merriman, Mac-  
 Donald & Evans, Ltd., London 1958 (p. 174 relied  
 upon).